

April 10, 1934.

W. H. FOWLE ET AL

1,953,932

TRAVELING KNIFE

Filed Feb. 28, 1933



*Fig. 2*



*Fig. 3*



*Fig. 4*



*Inventors*  
Walter H. Fowle  
Edward T. Leker  
Seymour Earle & Nichols  
*Atty*

## UNITED STATES PATENT OFFICE

1,953,932

## TRAVELING KNIFE

Walter H. Fowle, Woburn, Mass., and Elwood T. Ickes, Pittsburgh, Pa., assignors to John L. Fowle Company, Woburn, Mass., a partnership composed of Jessie A. Fowle, Edna Fowle, Florence Haley, and Walter H. Fowle

Application February 28, 1933, Serial No. 658,902

3 Claims. (Cl. 69—10)

This invention relates to traveling knives, and more particularly to endless or belt traveling knives of the type used for splitting leather, rubber and the like, and methods of making the same.

5 One object of this invention is to provide a traveling knife with a rear or thrust edge of such characteristics as to substantially prevent the development of cracks adjacent the thrust edge, thus permitting the knife to have a greater length 10 of useful life with corresponding economy.

Another object of this invention is to provide a traveling knife with a harder cutting edge than has heretofore been feasible in similar knives, and at the time to provide the thrust edge of the knife 15 with such characteristics as to substantially prevent the development of cracks adjacent the thrust edge.

The above and other objects will appear from the following description and appended claims 20 forming a part of this specification.

In the accompanying drawing:

Fig. 1 illustrates a plan view of a portion of an endless or belt knife used for splitting leather, rubber, and the like;

25 Fig. 2 is an edge view of Fig. 1;

Fig. 3 is a diagrammatic view of a knife being passed between heated rollers to reduce the hardness of the thrust edge portion of the knife; and

30 Fig. 4 is a similar view of a knife being passed through molten lead to reduce the hardness of the thrust edge portion of the knife.

In the art of splitting leather, rubber and the like, it is usual to have an endless or belt knife usually about  $3\frac{1}{4}$  inches wide and  $\frac{1}{8}$  inch thick 35 similar to the portion of the knife 10 illustrated in the drawing. The knife usually has a length of from 25 to 32 feet with the ends of the strip forming the knife abutted together and brazed to form an endless knife which extends around 40 two pulleys usually about 30 inches in diameter and suitably spaced apart horizontally from each other to hold the endless knife taut. One of the pulleys is power-driven to cause the endless knife to travel continuously in one direction.

45 The upper part of the knife traveling between the two spaced pulleys is the portion of the knife which is used for the splitting operation, the front edge 11 of the knife constituting the cutting or splitting edge and the rear or thrust edge 50 12 engaging or thrusting against a suitable fixed abutment to hold the knife in position against thrusting action of the leather or rubber against the cutting edge 11.

The traveling knife is made of very fine quality 55 steel such as razor steel and is given a suitable

hardness or temper for the work to be performed. The cutting edge of the knife dulls rather rapidly and is repeatedly resharpened until the width of the knife is reduced from its original width of  $3\frac{1}{4}$  inches to approximately  $1\frac{1}{4}$  inches, when it 60 is discarded. Usually, however, long before the knife has worn down to a width of  $1\frac{1}{4}$  inches, cracks such as 13 develop at the thrust edge 12 of the knife and progressively develop and extend toward the cutting edge 11 of the knife, thus resulting in the knife usually being discarded long 65 before it would be discarded if there were no serious cracks present.

These cracks appear to result from strains and from the rubbing of the thrust edge 12 of the 70 knife against the fixed abutment previously mentioned.

The steel used, usually contains from .60 to 1.20 per cent of carbon and may contain alloy such for example as nickel and/or chromium and/or 75 other metals. The range of temper given to the knife is usually from 35 to 46 C-Scale Rockwell. Temper 46 is preferably used by expert operators on hard dry leather. Temps below 46 down to 35 are used, depending on conditions, the softer 80 tempers being used on softer materials such as sheepskin and also being used by the less skilled operators to avoid danger of splitting the rear of the knife due to excessive strains brought on the knife.

85 We have discovered that by giving the portion of the knife extending along and adjacent the thrust edge 12, a temper suitably lower than the temper of the cutting portion of the knife, the development of cracks adjacent the thrust edge is 90 substantially prevented.

We have further discovered that by providing the portion of the knife extending along and adjacent the thrust edge with a temper which substantially prevents the development of cracks, the 95 hardness of the portion of the blade extending along and adjacent the cutting edge of the blade can be stepped up to provide a cutting edge of increased hardness, which is a matter of great commercial importance, since it enables an increased 100 output of split leather or rubber to be obtained due to the cutting edge remaining sharp for a longer period of time before requiring resharpening. The less frequent resharpening also results in the knife having a longer useful life, with corresponding economy. Knives made in accordance with our invention may be provided with the cutting portion from about 42 to 50 temper C-Scale Rockwell.

105 We preferably provide the thrust portion of 110

the knife with a temper above 27 but preferably not above 35 temper C-Scale Rockwell. The thrust portion of the blade which is given the low, anti-cracking temper is preferably a strip 5 from about  $\frac{1}{4}$  inch to about 1 inch in width extending along and adjacent the thrust edge. The remainder of the width of the knife is given the desired higher cutting temper.

In practice, the entire knife is preferably given 10 the desired high cutting hardness or temper in any desired way, and then the strip of desired width along the thrust edge 12 is given the desired, lower anti-cracking temper by suitable temper-drawing procedure, such as passing the 15 strip adjacent the thrust edge 12 between rollers 14 suitably heated, electrically or otherwise, or by passing it through suitably heated material 15 such as molten lead or the like.

The invention may be carried out in other 20 specific ways than those herein set forth without departing from the spirit and essential characteristics of the invention, and the present embodiments are therefore to be considered in all respects as illustrative and not restrictive, and all 25 changes coming within the meaning and equivalency range of the appended claims are intended to be embraced therein.

We claim:

1. A band traveling knife of considerable width 30 for splitting leather, rubber or the like comprising: a knife edge, a thrust edge, and a body intermediate said edges, said knife edge and the portion of the body at and extending back a considerable distance from the knife edge having a suitable substantially-uniform cutting hardness 35 greatly less than glass-hard, and a portion

of the body at and extending back from the thrust edge having substantially less hardness than the knife edge, whereby development of cracks adjacent the thrust edge is substantially prevented.

2. A band traveling knife of considerable width 40 for splitting leather, rubber or the like comprising: a knife edge, a thrust edge, and a body intermediate said edges, said knife edge and the portion of the body at and extending back a considerable distance from the knife edge having a suitable substantially-uniform cutting hardness 45 greatly less than glass-hard but substantially greater than 35 C-Scale Rockwell, and a portion of the body at and extending back a considerable distance from the thrust edge having substantially less hardness than 35 C-Scale Rockwell, whereby development of cracks adjacent the thrust edge is substantially prevented.

3. A band traveling knife of considerable width 50 for splitting leather, rubber or the like comprising: a knife edge, a thrust edge, and a body intermediate said edges, said knife edge and the portion of the body at and extending back a considerable distance from the knife edge having a suitable substantially-uniform cutting hardness 55 greatly less than glass-hard and at least 35 C-Scale Rockwell, and a portion of the body at and extending back from the thrust edge having less hardness than the knife edge and substantially 60 less than 35 but greater than 27 C-Scale Rockwell, whereby development of cracks adjacent the thrust edge is substantially prevented.

WALTER H. FOWLE.

110

ELWOOD T. ICKES.

40

115

45

120

50

125

.55

130

.60

135

65

140

70

145

75

150